

## UNITED STATES PATENT OFFICE

HENRY DREYFUS, OF LONDON, ENGLAND

## TREATMENT OF YARNS, FABRICS, FILMS, AND THE LIKE

No Drawing. Application filed January 19, 1927, Serial No. 162,215, and in Great Britain May 26, 1926.

This invention relates primarily to yarns or threads, or woven, knitted, or other textile fabrics or other materials made of or containing artificial filaments or fibres of cellulose acetate or other carboxylic acid esters of cellulose, for example, cellulose formate, butyrate or propionate, or cellulose esters, for example, methyl, ethyl or benzyl cellulose, or the corresponding condensation products of cellulose and glycols or other polyhydric alcohols, all of which are hereinafter referred to as organic substitution derivatives of cellulose. The invention also relates to ribbons, films or similar products made of the aforesaid organic substitution derivatives of cellulose.

It has recently been found that the aforementioned classes of textile and other goods made from or containing the aforesaid organic substitution derivatives of cellulose, and especially cellulose acetate, can be subjected to a loading or weighting operation, of the kind adopted for loading or weighting natural silk, without detriment to the permanence, strength or lustre of the goods and with marked advantage to certain of their other physical characteristics.

Thus the tendency of woven fabrics made of yarns of cellulose acetate or other of the aforesaid organic substitution derivatives of cellulose to slip, that is to say for the yarns to become displaced in the fabric, the tendency of circular knitted fabrics to "ladder", and the tendency of warp knitted fabrics to "split" are all considerably reduced and may even be practically eliminated.

The loaded goods can also be subjected to higher temperature than the unloaded goods without melting or becoming sufficiently plastic, to endanger their characteristic form or structure, so that for example, the possibility of damaging cellulose acetate and like fabric through using too hot an iron in ironing is lessened. The flammability of cellulose acetate or other goods of the classes previously specified, is likewise reduced. The fullness or volume of yarns or threads or woven, knitted, or other textile fabrics made from or containing artificial

filaments of cellulose acetate or other of the aforesaid substitution derivatives of cellulose is also improved.

The fact that goods composed of cellulose acetate or other of the aforesaid organic substitution derivatives of cellulose can be loaded in the same way as natural silk is of a somewhat surprising character in view of the well-known water-resisting properties of these goods, and the difficulties encountered in dyeing the same, but is no doubt closely associated with the swelling action which aqueous solutions of the agents—tannin, stannic chloride, etc.—employed for loading, or for the first stage of the loading operation, exert upon cellulose acetate and similar artificial silks.

It has now been discovered that the range of loading agents that can be used and the amount of loading effected in a single operation can be greatly extended if the goods are treated either initially or before or during or both before and during any stage of the loading operation with agents, for example, aqueous swelling solutions for cellulose acetate or other of the aforesaid organic substitution derivatives of cellulose, that impart to the filaments, films or like elementary structures whereof the goods are wholly or in part constituted a capacity or an increased capacity for absorbing the agents employed in loading.

More particularly, it has been found that the use of aqueous swelling-solutions containing solvents or swelling agents for cellulose acetate or other of the aforesaid organic substitution derivatives of cellulose give rise to a very considerable increase in the amount of loading that can be effected in a single operation or cycle of operations.

Especially advantageous results have been attained by the use of aqueous solutions of organic hydroxy compounds such as glycolic acid, lactic acid, ethyl alcohol, diacetone alcohol, diacetine, phenol, hydroquinone or other water soluble phenols or polyhydric phenols or acetone, or other water soluble organic solvents or swelling agents for the cellulose acetate or other cellulose derivative, or mixtures thereof.

In some cases, aqueous solutions of thiocyanates, particularly ammonium thiocyanate, or other salts acting as swelling agents may be employed; aqueous solutions containing mixtures of such salts together or with organic solvents or swelling agents may also be used.

It is to be understood that the solvent or swelling agent employed must not be used in such concentration or under such conditions as to dissolve the filaments, films or other elementary structures of cellulose acetate etc., or to endanger their characteristic form or structure or to damage their permanence, strength, lustre or other characteristics.

The loading may be effected by treatment with any loading agent that is capable of being absorbed by the filaments, films, etc. after they have been treated with solutions of solvents or swelling agents in accordance with the invention. Thus, the goods may be loaded with insoluble compounds or salts such as tannates, phosphates or silicates by two stage processes involving the use or application of an aqueous solution of a chloride or other soluble salt of a metal for example, tin, zinc, aluminum, bismuth, tungsten, antimony etc. preceded or followed by a solution of tannic acid, a phosphate, silicate or other precipitant for the metal.

The treatment with an aqueous solution of a solvent or swelling agent is usually applied before the loading operation proper, and may also with advantage be applied before each stage of the loading operation, or, when the cycle of loading operations is repeated, before each cycle or each stage of each cycle. Alternatively the solvent or swelling agent may be incorporated with each or all of the aqueous solutions used for loading. When one of the loading solutions used is itself a swelling solution, and particularly when it is a powerful swelling solution, the preliminary or simultaneous use of a nonloading solvent or swelling agent at that stage of the loading operation may be omitted.

The manner in which the invention can be carried into effect is described in the following examples, which are illustrative but not limitative in character.

#### Example 1

Woven or knitted fabric made from cellulose acetate artificial silk is soaked in a 7-10% solution of acetone for  $\frac{1}{2}$ -1 hour. The fabric is then steeped in a stannic chloride solution of 45-50° Tw. for half an hour and thoroughly rinsed. The fabric is again soaked in a 7-10% solution of acetone for about  $\frac{1}{2}$  hour, and is then treated in a solution of disodium phosphate of 4-6° Tw. at 40°-65° C. for  $\frac{1}{2}$  hour. The goods are afterwards rinsed and washed.

#### Example 2

Cellulose acetate fabrics or yarns are immersed in a 50% solution of alcohol, or a 15-20% solution of diacetone alcohol, for about  $\frac{1}{2}$  hour, and are then loaded with stannic chloride and disodium phosphate under similar conditions to those given in Example 1, with or without an intermediate treatment with a swelling solution, usually that employed for the initial treatment.

#### Example 3

Cellulose acetate fabrics are steeped in a 10-12% solution of ammonium thiocyanate preparatory to loading by successive treatment with a stannic chloride solution of 40° Tw. and a sodium silicate solution of 7° Tw. The goods are thoroughly rinsed after each treatment.

The goods may with advantage be washed in a soap solution after the loading operation is completed.

The amount of the loading depends upon a number of factors; of these, the most important is the extent to which the treatment with a swelling solution is adopted, the greatest effect being obtained when the goods are subjected to the action of a swelling solution before or during each stage of the loading operation. In general, an increased loading effect is obtained by the use of higher concentrations, whether of swelling or loading agents, or by prolonged treatment at each or any stage, while repetition of the cycle of operations leads to a very considerable improvement in the loading.

Care should however be taken not to use such concentrations, temperatures, swelling solutions, or other conditions or agents,—or to subject the goods to so many repetitions of the loading process,—as to produce tendering or loss of lustre or other undesirable effects on the character or quality of the goods.

The process forming the present invention may be applied to goods that are composed wholly of cellulose acetate or other of the aforementioned substitution derivatives of cellulose, or to mixed goods, for example, mixed fabrics containing yarns of wool, cotton, natural silk, artificial silk of the cellulose type, etc., or containing yarns composed of artificial filaments of cellulose acetate or other of the aforesaid organic substitution derivatives of cellulose doubled or associated with natural fibres, artificial silks of the cellulose type etc.

The invention also includes the loaded or weighted fabrics or other goods produced in accordance with the invention.

What I claim and desire to secure by Letters Patent is:—

1. Process for treating material comprising artificial filaments of organic deriva-

ties of cellulose, comprising subjecting the material to the action of a swelling agent comprising diacetone alcohol and loading the material by fixing an insoluble metallic compound therein.

2. Process for treating material comprising artificial filaments of organic derivatives of cellulose, comprising treating the material with a swelling agent containing diacetone alcohol, and with a loading agent and then fixing the loading agent.

10 3. Process for treating material comprising artificial filaments of cellulose acetate, comprising subjecting the material to the action of a swelling agent comprising diacetone alcohol and thereafter loading the material by fixing an insoluble compound of a heavy metal therein.

20 4. Process for treating materials comprising artificial filaments of organic derivatives of cellulose, comprising subjecting the material to the action of a swelling agent comprising diacetone alcohol and thereafter loading the material by fixing an insoluble compound of a heavy metal therein.

26 5. Process for loading materials comprising artificial filaments of organic derivatives of cellulose, comprising treating the material with a swelling agent comprising diacetone alcohol and with a solution of a salt of a heavy metal, again treating the material with a swelling agent, and thereafter fixing the heavy metal in the material as an insoluble compound.

35 6. Process for loading materials comprising artificial filaments of cellulose acetate, comprising treating the material with a swelling agent containing diacetone alcohol and with a solution of a salt of a heavy metal, again treating the material with a swelling agent comprising an organic hydroxy compound, and thereafter fixing the heavy metal in the material as an insoluble compound.

45 46 In testimony whereof I have hereunto subscribed my name.

HENRY DREYFUS.

**CERTIFICATE OF CORRECTION.**

**Patent No. 1,821,464.**

**Granted September 1, 1931, to**

**HENRY DREYFUS.**

**It is hereby certified that error appears in the printed specification of the above numbered patent requiring correction as follows: Page 3, lines 41 and 42, claim 6, strike out "an organic hydroxy compound" and insert instead diacetone alcohol; and that the said Letters Patent should be read with this correction therein that the same may conform to the record of the case in the Patent Office.**

**Signed and sealed this 27th day of October, A. D. 1931.**

**(Seal)**

**M. J. Moore,  
Acting Commissioner of Patents.**